

## UNITED STATES PATENT OFFICE

2,179,066

## MANUFACTURE OF SULPHURIZED SPERM OIL

Herschel G. Smith, Wallingford, Pa., assignor to  
Gulf Oil Corporation, Pittsburgh, Pa., a corporation of PennsylvaniaNo Drawing. Application October 29, 1936,  
Serial No. 108,306

15 Claims. (Cl. 260—327)

This invention relates to the manufacture of sulphurized sperm oils and like esters, and it comprises methods of making such sulphurized esters wherein sperm oils and like unsaturated mono-

5 esters of fatty acids are sulphurized and substantially neutral organic compounds are obtained, the sulphurization being gradually effected, advantageously by gradually adding sulphur to pre- heated sperm oil and maintaining the mixture be-

10 tween 300 and 385° F. until substantially all the sulphur has combined, and it also comprises the substantially neutral sulphurized sperm oils so obtained, said sulphurized oils being soluble in and

15 miscible with petroleum oils and like hydrocarbons and useful as improvement agents for petroleum products and being capable of imparting extreme pressure characteristics to mineral lubricating oils and other lubricants and of improving the other properties of such petroleum products; all as more fully hereinafter set forth and as claimed.

20 In my copending application Serial No. 60,355, filed January 22, 1936, I have described and claimed improved lubricants containing sulphurized sperm oils and like sulphurized esters and methods of making such lubricants, which applica-

25 tion is a continuation-in-part of my application Serial No. 715,551, filed March 14, 1934, now U. S. Patent No. 2,056,247. The present application is a continuation-in-part of my said prior applica-

30 tions.

The present invention is directed to the sulphurized sperm oils and to methods of making the same wherein sulphur is reacted and chemically combined with sperm oil and like unsaturated aliphatic mono-esters of an unsaturated aliphatic mono-ovalent acid and an unsaturated aliphatic mono-ovalent alcohol, to produce substantially neutral organic sulphides readily soluble in mineral oils.

40 The sulphurization of fatty oils is well known, the usual practice being to mix relatively large amounts of sulphur with the fatty oil and heat the mixture until a sulphurized fatty oil is obtained. Such sulphurized fatty oils have been used for many purposes in the industrial arts. For instance, sulphurized fatty oils, obtained by adding sulphur to a fatty oil such as lard oil, etc. and heating the mixture for several hours, have been frequently used in making the so-called cutting oils. Such cutting oils are primarily mix-

tures of mineral oil with sulphurized fatty oils. These oils and other mixtures of mineral oil and sulphurized fatty oil are well known in various arts.

Likewise, it is well known that the addition of sulphurized oil to mineral oils, imparts extreme pressure characteristics to them. There being a demand for lubricants which in the form of thin films are capable of withstanding high pressures, such as occur in the gear and transmission combination of modern automobiles and other machines, it has been proposed to use mixtures of mineral oil and sulphurized fatty oil for lubricating such machines. However, it has been found that the usual mixtures are not sufficiently stable in storage or in use or both and that they are more corrosive than is permissible.

The ordinary fatty oils or esters heretofore employed for said purposes are glycerides; they being tri-esters of glycerine in which the glycerine is esterified with three mols of fatty acid. I have found that it is somewhat difficult to control the sulphurization of such tri-esters and that many of the sulphurized products obtained from them are not suitable for blending with lubricating compositions for several reasons. For one thing, they frequently lack sufficient solubility for blending with many of the usual lubricating bases. Again, when sufficiently soluble to permit blending with mineral oil under some conditions, they are insufficiently miscible over a range of conditions to permit the production of good stable compounded lubricants. Further, many of the mixtures of sulphurized tri-esters of fatty acids and mineral oils are often corrosive to various metals and alloys such as used in gears and bearings, particularly certain alloys such as binary and ternary alloys of silver, cadmium, nickel, copper and lead. In many cases this corrosiveness, while not apparent in the freshly prepared compounded lubricant, develops during storage or in use.

Although sperm oil is frequently termed a fatty oil, it is quite different from the ordinary fatty oils, which are tri-esters of glycerine. Sperm oil is composed principally of the fatty esters of monohydric alcohols of relatively high molecular weight; it being a mono-ester. Actually sperm oil is a liquid wax of the ester type. Being an ester, it is also different from the paraffin hydrocarbons commercially known as waxes.

5

10

15

20

25

30

35

40

50

Sperm oil is obtained from the head cavities and blubber of the cachalot or sperm whale (*Physeter macrocephalus*). The crude oil contains varying amounts of spermaceti and like solid waxes of the ester type. In refining the oil, these waxes are removed by refrigeration and pressing, to obtain the commercial sperm oils. The commercial oils are known as winter sperm oil, spring sperm oil, etc., and are substantially free of solid waxes. The commercial sperm oil is a thin yellow liquid and when of good quality is nearly free from odor. In the present invention it is advantageous to use refined sperm oil of good quality.

Sperm oil itself is a good lubricant. Being both 15 limpid and substantially free from any tendency to "gum" (usually resistant to oxidation and resification), it has been long used to lubricate light machinery. Also, it has been blended with mineral oil to form compounded lubricants.

20 I have found that by controlledly sulphurizing sperm oil, its lubricating qualities are enhanced. The sulphurized sperm oils so prepared, have desirable viscosities and blending properties which render them exceedingly useful in compounding 25 lubricants. They may be compounded with lubricating mineral oils and various other lubricating compositions according to the procedures set forth in my companion application Serial No. 60,355 to obtain improved lubricants.

30 By the present invention there are readily obtained sulphurized sperm oils and like esters for many industrial purposes. Excellent sulphurized esters advantageous as improvement agents for lubricants may be readily prepared, for instance, 35 the advantageous sulphurized sperm oils having the following properties:

|                                       |           |
|---------------------------------------|-----------|
| Gravity, °A. P. I.                    | 13.6-14.6 |
| Viscosity, S. U. V., 210° F., seconds | 200-300   |
| Pour, °F. (not greater than)          | +45       |
| 40 Sulphur, per cent                  | 8-14      |
| Neutralization number                 | 1-1.5     |

Sulphurized sperm oils having the above properties are readily soluble in all of the ordinary 45 grades of lubricating oils. They are fully miscible and compatible with the high gravity mineral oils, such as paraffinic base oils (Pennsylvania, etc.) and solvent refined oils, etc., over a wide range of conditions such as temperature, proportions, etc. 50 When they are compounded with such mineral oils, improved compounded lubricants are obtained which are remarkably stable, as well as having viscosities, viscosity indexes, specific gravities, pour points, etc., capable of meeting the 55 technical specifications for high grade commercial lubricants. Their lubricating qualities over a wide range of utilization are excellent.

To produce such high grade sulphurized oils I find it is advantageous to use, as the starting material, commercial sperm oil having the following 60 properties, for example, but not by way of limitation:

|                                   |             |
|-----------------------------------|-------------|
| Specific gravity, 60°/60°F        | 0.878-0.884 |
| Viscosity, S. U. V., 100° F.      | 95-110      |
| 65 Flash, O. C., °F., minimum     | 490         |
| Pour, °F., maximum                | +40         |
| Color, N. P. A., not darker than  | 1.5         |
| Neutralization number, maximum    | 0.5         |
| Oleic acid eq., per cent, maximum | 0.25        |
| 70 Saponification number          | 125-135     |
| Iodine number                     | 80-90       |

The sulphur employed should be of good quality and free of any abrasive material such as sand, fossil fragments, etc. Sublimed sulphur,

such as flowers of sulphur, is advantageous. However, any finely ground sulphur, such as sulphur flour, may be used.

The amount of sulphur used to sulphurize the sperm oil may be varied according to the particular sperm oil being processed and the specific characteristics desired in the final product. Usually the ratio of sulphur to oil is between 5:95 and 20:80. Generally, I employ substantially an amount of sulphur not exceeding that necessary to 10 saturate the double bonds of the sperm oil used. In controlling the ratio of sulphur to oil, some unsulphurized sperm oil may be present in the final product. This is permissible as unsulphurized sperm oil is more or less a desirable 15 and advantageous ingredient in certain lubricating compositions.

By properly controlling the sulphurizing operation, for instance, by employing the methods given post, the percentage of combined sulphur 20 in the sulphurized sperm oil is approximately that in the reaction mixture. Likewise, very little hydrogen sulphide is formed when the reaction is properly controlled.

In preparing the sulphurized sperm oil, the 25 sperm oil is reacted with suitable amounts of sulphur at temperatures between about 300-385° F., the reaction being continued until the sulphur is combined in the form of neutral organic sulphur compounds. However, to obtain superior 30 sulphurized sperm oils, I find it advantageous to use reaction temperatures between 335° and 360° F. and to employ controlled methods of sulphurization, wherein decomposition of the oil, side reactions, over-vulcanization, etc., are substantially avoided. If the sulphurization is properly conducted, the viscosity of the oil sharply increases and then the viscosity tends to become 35 substantially constant during the remainder of the heating.

In general, control of the sulphurization is obtained by first preheating the sperm oil to about the lower reaction temperature (325° F.) or slightly below, and then gradually adding the required amount of sulphur to the preheated oil, the 45 rate of addition being adjusted so that heat developed during the addition of the sulphur gradually and quietly raises the reaction mixture to a temperature just below the preferred upper limit (360° F.). Advantageously, the finely divided sulphur may be gradually sifted into the oil while 50 agitating. After all the sulphur has been added, the temperature tends to drop slightly and then the reaction mixture is maintained at about 345° F. until the reaction is complete. The course 55 of the reaction may be easily followed by withdrawing test samples and determining the change in viscosity. After the proper viscosity has been obtained, the end point can easily be determined by diluting the sulphurized oil with a standard 60 amount of mineral oil and determining its corrosive action upon a copper strip. When the copper strip remains unattacked or shows only a slight stain, the reaction is complete. Then the sulphurized oil is cooled to about room temperature. It can be stored in metal drums or other 65 suitable containers.

The copper strip test here employed was devised by me in 1917 for determining the relative corrosiveness of lubricating oils. The procedure is 70 as follows:

A mechanically polished copper strip  $\frac{1}{2}$  inch by 3 inches is immersed in 25 cc. of lubricant contained in a test tube which is placed in a boiling water bath and held at the temperature of boil- 75

ing water for three hours. At the end of this time the strip is removed and adhering oil washed off with a light naphtha and examined for evidence of corrosion. A negative test is one in which the 5 strip shows only a slight stain or discoloration. The positive test is one where the strip shows considerable discoloration or tendency to scale, indicating presence of corrosive constituents in the lubricant.

10 In preparing the diluted sample for a test, I ordinarily use a standard mineral oil having the following properties:

|                              |        |
|------------------------------|--------|
| Gravity, A. P. I.            | 27.1   |
| Specific gravity, 60°/60° F. | 0.8922 |
| Viscosity, S. U. V., 100° F. | 1059   |
| Viscosity, S. U. V., 130° F. | 420    |
| Viscosity, S. U. V., 210° F. | 89     |
| Viscosity index              | 92     |
| 20 Flash, O. C., °F          | 470    |
| Fire, O. C., °F              | 545    |
| Pour, °F                     | +5     |
| Color, N. P. A. (dil.)       | 4.25   |
| Carbon residue, per cent     | 0.44   |
| 25 Neutralization number     | 0.01   |

The sample of sulphurized sperm oil is diluted with the above mineral oil in the ratio of 10:90 to obtain the sample used in determining the corrosion by the copper strip method. The copper 30 strip is removed from the heated oil sample after 3 hours, and then wiped dry and inspected in the usual manner. Sometimes, a test mixture the same as the desired compounded lubricant is used in the above test.

35 With the above mentioned controlled methods of sulphurization, there is but little loss of sulphur; the percentage of combined sulphur in the sulphurized sperm oil is approximately that in the reaction mixture. During the sulphurization, 40 very little hydrogen sulphide is formed. As the finely divided sulphur is gradually added to the hot oil by sifting, etc., there may be more or less mechanical loss of sulphur. With careful operation, however, this loss may be minimized, if not 45 entirely avoided.

The viscosity of the oil increases rather rapidly as the sulphur is added and upon combination of most of the sulphur the viscosity tends to remain substantially constant as the heating is 50 continued. Undesirably low reaction temperatures should be avoided for the best combination of the sulphur and exceedingly high temperature should be avoided to prevent undesirable side reactions. By way of specific example as to the 55 heating, with the sperm oil preheated to between 325-340° and the sulphur gradually added so as to bring the reaction temperature to between 330 and 360° F., the maximum viscosity is obtained with 6 to 11 hours heating; all the sulphur 60 being added during the first two hours. Upon maintaining the temperature at 340±5° F., all the sulphur can be brought into combination in the form of neutral sulphur compounds within 16 to 24 hours, with but a slight decrease in the viscosity during digestion. Thus by following the 65 reaction by means of viscosity tests upon test samples withdrawn from the batch and by means of corrosion test made at about the end point, satisfactory sulphurized sperm oil may be readily 70 and consistently produced by my improved method; the details of ratios of sulphur to oil, of rate of addition of sulphur and of time of heating being adjusted to the particular materials and equipment used in commercial practice.

75 From the description ante, the ranges of tem-

perature generally used are between 325 and 360° F. and the time of heating is between 16 and 24 hours, the sulphur being added during the first two hours. After the reaction is completed, the sulphurized oil is cooled to room temperature and, if desired, may be filtered or screened to remove any foreign bodies or abrasive materials that may have been accidentally introduced into the batch. As the sulphurized sperm oil is quite viscous, the filtration may be made while the oil is still hot. Sometimes the sulphurized oil may be centrifuged, but ordinarily this is unnecessary when care has been used to exclude introduction of foreign matter. However, centrifuging can be advantageously used in later stages of the 10 processing as shown post.

The controlled method of sulphurization here employed has several advantages. By first pre-heating the sperm oil, it is more or less dried during that step; the water and other volatiles being evaporated. Removal of these volatiles helps to minimize side reactions and the production of corrosive sulphur compounds. Further, the sulphur more readily dissolves in the hot oil and a uniform mixture of the reactants is quickly 15 and readily obtained. Stratification of a heavy layer of molten sulphur and oil, frequently encountered in sulphurizing fatty oils, can be entirely avoided by the present methods. The sulphur being added in finely divided form to the so-heated oil becomes converted into molten drops which completely dissolve in the oil before they have time to settle to the bottom of the reaction vessel. As the mixing is performed at reaction 20 temperature, combination of the sulphur with the oil in the desired manner is immediately initiated and thus a high yield of neutral sulphur compounds is obtained. Likewise, the time of reaction is held to a minimum and decomposition of the oil and of the neutral sulphur compounds 25 is avoided. Again, the elevated temperature used throughout the operation renders the sulphurized oil, as formed, more mobile thus facilitating the addition and mixing of the last portions of the sulphur. In accomplishing this result, the heat 30 of reaction is permitted to increase slightly the temperature of the reaction mixture in the first stages. In turn, many of these advantageous results may be attributed to the gradual addition of the sulphur in the manner set forth ante. In 35 this controlled method there is a worthwhile 40 overall efficiency leading to a high yield of desirable sulphurized sperm oil of high purity with a minimum loss of materials.

The sulphurized sperm oil here obtained, by 45 gradual sulphurization, when added to mineral oil in minor amounts yields improved compounded lubricants. It may be advantageously compounded with any of the ordinary mineral lubricating oils to modify the properties thereof. 50 Varying amounts of sulphurized sperm oil may be employed according to the compounded lubricant desired and the mineral oil base used. By blending from one-tenth per cent to thirty per cent by weight of sulphurized sperm oil with the 55 various types of lubricating oils and greases, I obtain a wide range of commercial lubricants 60 wherein one or more properties of the lubricant are advantageously improved.

In my copending applications Serial Nos. 60,355 70 and 60,357, there are given numerous illustrative embodiments of such commercial blended lubricants containing sulphurized sperm oil and like mono-esters. My application Serial No. 60,357 filed January 22, 1936, is directed to improved 75

lubricants containing sulphurized mono-esters of fatty acids.

Also the sulphurized sperm oils obtained by the present invention may be used in making improved pipe thread lubricants as disclosed in my copending application Ser. No. 60,356, (now Patent No. 2,065,248) filed January 22, 1936, that application being directed to such improved thread lubricants.

10 As stated ante, in lieu of sperm oil itself (oil from the cachalot whale) other "oils" of the sperm oil group may be used in making the sul-  
phurized products according to this invention.  
For instance, bottlenose oil (doegling oil) may be  
15 employed. It is obtained from several species of  
toothed cetaceans, particularly the bottlenose  
whale (*Hyperoodon rostratum*); hence the name  
of "bottlenose oil". It is so like true sperm oil  
in character, that the commercial oil is known as  
20 arctic sperm oil. The said class of oils have cer-  
tain properties in common with true sperm oil;  
all of these oils containing characteristic types of  
fatty esters.

As is well known, true sperm oil is a mixture of certain esters. Those esters are the esters of monohydric alcohols with fatty acids of the oleic series, such esters having the following general formula,



wherein R represents an aliphatic chain of relatively high molecular weight; the acid component being likewise of high molecular weight. From the information available, such as reported analysis, the principal and characteristic components of sperm oil and similar oils of the sperm oil group are mono-esters which are unsaturated or contain double bonds, on each side of the ester group. That is, they are esters of oleic acid or homologous acids of the oleic type with monohydric alcohols of the ethylene series (the series of alcohols corresponding to the oleic series of acids). This characteristic class of mono-esters may be represented by the following formula:



50

wherein  $n$  is at least 1.

Commercial sperm oil contains minor amounts of other fatty esters but the above mentioned class of esters are the characteristic components thereof. Thus any oil and mixture of esters containing the said characteristic esters are useful in the present invention. Such esters may be sulphurized to form neutral organic sulphur compounds, which are advantageous in making compounded lubricants as set forth ante. For the present purposes, esters of this class which have a relatively high molecular weight are advantageous. That is, the sub-class of esters having the following formula:



wherein  $x$  is 1 to 7, are advantageous for making the said neutral sulphurized products. In sulphurizing them by the present methods, the add-

ed sulphur saturated the double bonds of such esters yielding products having neutrally combined sulphur in each half of the ester. Taking the oleate of oleyl alcohol (oleyl ester of oleic acid) wherein the said  $x$  of the above formula is 5, as an illustration, the neutral product may be represented by the following formul:



The following examples are illustrative embodiments of the methods broadly set forth ante and are not limitative of the invention.

*Example 1.*—This example illustrates an advantageous method of making the sulphurized sperm oil. A sperm oil having the following properties:

|                              |        |
|------------------------------|--------|
| Gravity, °A. P. I.           | 29.0   |
| Specific gravity, 60°/60° F. | 0.8816 |
| Viscosity, S. U. V.:         | 25     |
| 70° F.                       | 171    |
| 100° F.                      | 100    |
| 130° F.                      | 71     |
| 210° F.                      | 43.3   |
| Flash, O. C., °F.            | 505    |
| Pour, °F.                    | +35    |
| Color Saybolt                | -5     |
| Neutralization number        | 0.14   |
| Saponification number        | 130.9  |
| Iodine number                | 87     |

was sulphurized under controlled conditions, using approximately 12 per cent sulphur by weight on the oil.

40  
45  
50  
55  
Weight 11.1  
Into a direct-fired, 20-barrel, open-top grease kettle I charged 8057 lbs. of said sperm oil (1097 gal.) and gradually heated the oil to 320° F. in about 4 hours, while stirring. While continuing the stirring, 1098 lbs. of sulphur flour (approximately 1 lb. of sulphur per gallon of oil) was gradually added by sifting it into the hot oil over a period of two hours and at such a rate as to maintain a steady increase in temperature to 360° F. Then the temperature was gradually lowered to 340° F. and the reaction mixture maintained at that temperature and stirred for 16 hours; the heating then being stopped and the sulphurized oil cooled to normal temperature. The total time from the first addition of sulphur to the completion of the reaction was about 20 hours.

In the above type operation, after the reaction has been initiated, the fire may be drawn or cut off during the addition of the rest of the sulphur, but usually it is only lowered so as to prevent undue loss of heat by radiation. After the reaction mixture is brought to 340° F., the fire is increased to hold that temperature during the remainder of the reaction. The change in viscosity during the reaction was as follows:

| After first addition of sulphur, hours | Viscosity, S.U.V.<br>at 210° F.,<br>seconds |
|----------------------------------------|---------------------------------------------|
| 1                                      | 68                                          |
| 2                                      | 177                                         |
| 4                                      | 267                                         |
| 8                                      | 276                                         |
| 12                                     | 268                                         |
| 16                                     | 242                                         |

Operating in this way, there was obtained 9064 lbs. of sulphurized oil; the percentage yield by weight being 99.0 per cent of the materials charged. As part of the loss is due to evaporated water and other volatiles from the sperm oil and sulphur, clearly only a very small amount of H<sub>2</sub>S is formed. During the sulphurization a slight odor of hydrogen sulphide was detectable, but the sulphurized oil did not have an objectionable odor. During sulphurization the oil increased in volume and the yield by volume was 1120 gallons. The sulphurized oil so obtained was of high quality and had the following properties:

|                              |        |
|------------------------------|--------|
| 15 Gravity, °A. P. I.        | 14.1   |
| Specific gravity, 60°/60° F. | 0.9718 |
| Pounds per gallon            | 8.093  |
| Viscosity, S. U. V., 210° F. | 242    |
| Pour, °F.                    | +45    |
| 20 Sulphur (B), per cent     | 11.10  |
| Neutralization number        | 0.63   |
| Color, N. P. A.              | Dark   |

It is readily soluble or dispersible in mineral oil of various grades. When diluted with 90 parts of mineral oil to 10 parts of sulphurized oil, the diluted oil gave only a slight tarnish by the copper strip test.

In the above example the ratio and other details may be varied as indicated in the general description ante to obtain various specific products. In lieu of the particular sperm oil employed in Example 1, other unsaturated mono-esters of fatty acids, such as mentioned ante may be employed.

35 For instance, any of the following esters which are typical and illustrative of the same general class of fatty mono-esters, may be employed:

|    |                      |
|----|----------------------|
| 40 | Allyl oleate         |
|    | Decylene oleate      |
|    | Dodecylene oleate    |
|    | Pentadecylene oleate |

That is, in the broad practice of this invention there may be employed esters having the following formula:



50 wherein both R<sub>2</sub> and R<sub>3</sub> are olefinic aliphatic chains. Such esters are unsaturated (contain double bonds) in both the acid and alkyl components thereof. Generally, the esters of oleic acid and other mono-carboxylic acids of the oleic series with unsaturated mono-hydric wax alcohols may be employed. The acids of an unsaturated aliphatic mono-carboxylic acid are esterified with the corresponding alcohols and are, so to speak, balanced esters. The oleates of oleyl alcohol is typical of such balanced esters. However, the alcohol component of the ester does not necessarily have to correspond with the acid components thereof. The oleates of any of the oleyl alcohols present in sperm oil may be used.

65 The oleates are satisfactory and are ordinarily employed. Also, in lieu of natural mixtures of such esters, such as sperm oil, etc., any ester or mixture of esters of the general class set forth ante may be employed. That class is representative of the characteristic esters as sperm oil. That is, I may employ artificial or synthetic sperm oils comprising a mixture of such esters, in lieu of the sperm oils directly obtained from natural sources. In this way, the properties of the starting material and sulphurized products

obtained may be controlled to obtain sulphurized esters useful for special purposes.

By the procedure of Example 1, various sulphurized sperm oils and like mono-esters having the following properties:

|                              |           |
|------------------------------|-----------|
| Viscosity, S. U. V., 210° F. | 200-300   |
| Sulphur, per cent            | 10.0-12.1 |

may be readily obtained and these are advantageous as improvement agents for various mineral lubricating oils and petroleum lubricants.

Example 2.—This example illustrates the sulphurization of a simple balanced ester.

The oleate of oleyl alcohol is sulphurized at 15 temperatures between 325 and 360° F. with about 12 per cent of sulphur by weight on the said oleate, by reacting 500 parts of said oleate with 60 parts of sulphur. There is obtained a sulphurized mono-ester containing 10.7 per cent of 20 sulphur and having a viscosity S. U. V. at 210° F. of approximately 200-300.

The oleate of dodecylene alcohol may be likewise sulphurized. This oleate required 14.38 per cent sulphur to convert it into a substantially 25 neutral sulphide containing 12.5 per cent combined sulphur. In practice a good product is obtained by sulphurizing 100 parts of this oleate with 14 parts sulphur. Again the decylene acid ester of decylene alcohol may be employed. It 30 requires 17.0 per cent of sulphur on the ester to convert it into a substantially neutral sulphide containing 14.9 per cent of combined sulphur.

While in the foregoing examples I have described direct sulphurization of the sperm oil, I 35 at times find it advantageous to sulphurize sperm oil in the presence of another oil, as for instance a petroleum hydrocarbon oil which may well be the same as the oil used for the base for manufacturing the compound lubricant. That is, 40 some of the mineral oil is mixed with the sperm oil prior to the addition of the sulphur.

When a mixture of sulphurized esters is to be employed, I sometimes blend together two or more sulphurized products, instead of sulphurizing a mixture of esters. In this way a more direct control and adjustment of the properties of the sulphurized material, for addition to special lubricants, may be obtained.

55 In this specification and the claims, the term "sulphurizing" means sulphurizing with sulphur itself, that is, reacting and chemically combining sulphur with the aliphatic mono-esters set forth ante. Likewise in this specification and claims the "sulphurized" esters are those containing the sulphur in chemical combination with the mono-ester. These sulphurized mono-esters are free of chlorine and are substantially neutral organic sulphides. That is, the processes and 60 products of this invention are characteristically different from the sulphochlorinated fatty oils and esters obtainable by reacting sulphur chloride with fatty oils, etc.

What I claim is:

1. A composition of matter comprising the reaction product of sperm oil and elemental sulphur.

2. As a new product, a sulphurized aliphatic mono-ester comprising the reaction product of 70 sulphur and an aliphatic mono-ester of an unsaturated aliphatic monovalent acid and an unsaturated aliphatic monovalent alcohol, said sulphurized mono-ester containing combined sulphur in both of the aliphatic chains of the 75

acid and alcohol components thereof and said sulphurized ester being a substantially neutral organic sulphide and being free of chlorine.

3. As an improved oil, useful in making lubricants, a sulphurized sperm oil, said sulphurized sperm oil being a mixture of substantially neutral organic sulphides readily soluble in mineral oils and capable of improving the lubricating qualities of such mineral oils when dissolved therein in small amounts and being free of chlorine.

4. As an improved oil, useful in making lubricants, a sulphurized sperm oil having the following properties:

15 Gravity, °A. P. I. 13.6-14.6  
Viscosity, S. U. V., 210° F. 200-300  
Pour, °F. +45  
Sulphur, per cent. 8-14  
Neutralization number. 1-1.5

20 said sulphurized oil being a mixture of substantially neutral organic sulphides, being readily soluble in mineral oils and being free of chlorine.

5. As a new product, a sulphurized fatty mono-ester comprising the reaction product of sulphur and an unsaturated aliphatic mono-ester having the following formula:



30 wherein  $R_2$  and  $R_3$  are olefinic aliphatic groups, said sulphurized mono-ester being a substantially neutral organic sulphide containing combined sulphur in each of said aliphatic groups and being free of chlorine.

6. As a new product, a sulphurized fatty mono-ester comprising the reaction product of sulphur and dodecyne oleate.

7. As a new product, a sulphurized fatty mono-ester comprising the reaction product of sulphur and the oleate of oleyl alcohol.

8. In the manufacture of improved sulphurized oil products, the process which comprises pre-heating sperm oil to a temperature between 325 and 360° F., gradually adding finely divided sulphur to the hot oil and maintaining the reaction mixture at said temperature until a substantially neutral sulphurized oil is obtained.

9. The process of claim 8 wherein from 5 to 20 per cent sulphur is so added to the hot oil, the sulphur being added at such a rate as to maintain the temperature during that time at about 360° F., thus producing a superior sulphurized oil.

10. The process of claim 8 wherein the said

sperm oil used as the starting material has the following properties:

|                                   |             |
|-----------------------------------|-------------|
| Specific gravity, 60°/60° F.      | 0.878-0.884 |
| Viscosity, S. U. V., 100° F.      | 98-110      |
| Flash O. C., °F., minimum         | 490         |
| Pour, °F., maximum                | +40         |
| Color, N. P. A., not darker than  | 1.5         |
| Neutralization number, maximum    | 0.5         |
| Oleic acid eq., per cent, maximum | 0.25        |
| Saponification number             | 125-135     |
| Iodine number                     | 80-90       |

said oil being substantially free of solid waxes.

11. In the manufacture of sulphurized mono-esters, the improvement which comprises sulphurizing a fatty mono-ester having the following formula



20

wherein  $R_2$  and  $R_3$  are olefinic aliphatic groups, by chemically combining said mono-ester with sulphur in an amount not exceeding that necessary to saturate the double bonds in said olefinic groups to obtain substantially neutral organic sulphides readily soluble in mineral lubricating oil.

12. The process of claim 11 wherein said unsaturated aliphatic mono-ester is the oleate of oleyl alcohol.

13. The process of claim 11 wherein said unsaturated aliphatic mono-ester is dodecyne oleate.

14. In the manufacture of stable, sulphurized mono-esters, the process which comprises sulphurizing an unsaturated fatty mono-ester having the following formula:



40

wherein  $x$  is 1 to 7, by chemically combining said mono-ester with sulphur to saturate the double bonds of said ester and obtain a substantially neutral organic sulphide readily soluble in mineral lubricating oil.

15. As a new composition of matter, a stable addition product of sulphur and a naturally occurring unsaturated ester of a monohydric alcohol and a high molecular weight fatty acid, said sulphurized ester being free of chlorine and being a substantially neutral organic sulphide.

HERSCHEL G. SMITH. 55